

# UNITED STATES PATENT OFFICE.

RICHARD F. DALTON, OF NEW YORK, N. Y.

## ARTIFICIAL-FUEL COMPOSITION AND PROCESS.

1,260,286.

Specification of Letters Patent. Patented Mar. 19, 1918.

No Drawing.

Application filed January 12, 1918. Serial No. 211,628.

To all whom it may concern:

Be it known that I, RICHARD F. DALTON, a citizen of the United States, and resident of New York, borough of Bronx, in the county of Bronx and State of New York, have invented certain new and useful Improvements in Artificial-Fuel Compositions and Processes, of which the following is a specification.

10 Various attempts have been made to utilize coal dust and screenings, particularly from anthracite, as a fuel whereby the vast accumulations of this material may be substituted for the more expensive forms of fuel 15 such as coal or oil. The dust or screenings cannot be used alone in the ordinary furnace, due to the fact that large quantities fall directly through the grates to the ash-bed and a considerable portion is carried up the stack, 20 making a dense smoke, wasteful of fuel.

The mixing of the anthracite dust or screenings with ingredients acting as a binder and the compression of the product into briquets possesses certain advantages, 25 but involves the use of expensive labor and mixing and pressing machinery, bringing the cost sufficiently high to prevent the effecting of any material economies over the use of bituminous coal.

30 The addition of binders, such as clay or other noncombustible substances, whether the mixture be compressed or burned loose, often results in the formation of clinkers and in any event involves a loss of the heat 35 required to bring such inert substances up to the temperature of the fire-bed.

As a result of my invention or discovery, I am able to use commercial anthracite dust or screenings without adding expensive ingredients and without the use of expensive 40 mechanical operations such as grinding or pressing. I accomplish this result by adding thereto a comparatively small quantity of a combustible liquid of such a character that 45 it may be quickly, easily and economically mixed with the dust or screenings and which, at the same time, will act to hold together the small particles of coal forming the coal dust or screenings after the latter 50 are thrown on the fire-bed and while they are being heated up to the temperature of the free combustion of coal.

It is important that the liquid shall be 55 of low viscosity so that it will flow freely throughout the mass during the mixing and will merely wet the surface of the coal par-

ticles without filling the spaces between them. It is also important that the liquid shall be of high flash and boiling points so that it will remain in the coal dust for some 60 time after the latter is thrown on the fire and will burn with the coal dust, or at least will not all volatilize or burn out before the coal dust is heated up to such a temperature 65 that it begins to freely burn.

The coal dust or screenings which I employ are the commercial anthracite dust or screenings just as they come from the coal yards or mine dumps and without grinding or crushing. The particles of such dust or 70 screenings are substantially non-absorptive of liquid and vary in size from the finest powder to pieces of the size constituting what is known as "buckwheat" coal. The relative proportions of the finer and coarser 75 particles also vary; in some cases, the coarser particles predominating to such an extent as to make the screenings little or no different from the finer grades of "buckwheat" 80 coal.

The low viscosity liquid, in wetting the surfaces of the particles, loosely holds them together more by surface tension than by any adhesive properties of the liquid which are substantially negligible, due to the low 85 viscosity. Thus, the voids are not filled with liquid at least to any substantial or material extent, and the presence of the liquid does not interfere with the free passage of air therethrough during the burning.

I am aware that attempts have been made to produce an artificial fuel composed only of coal dust and a combustible liquid, but so far as I know, it has heretofore been considered necessary to either grind the coal 90 dust to a powder or use a high viscosity oil, or do both, which prevents the advantageous results and economies effected by means of my composition.

As a preferred liquid fuel for use with 100 the unground, substantially non-absorptive, commercial anthracite dust or screenings, I employ a liquid fuel formed as one of the waste or by-products in the manufacture of illuminating or heating gas. This liquid is 105 not only combustible but is of sufficiently low viscosity as to facilitate its ready mixture with the coal particles, but it is also of the desired high flash and boiling points. The analysis of a large number of samples 110 of the particular liquid which I have been using shows an average specific gravity of

1.06 and 17,018 B. T. U. per pound. Although I do not wish to be limited to this specific liquid, yet it is important that the liquid used have the general properties hereinbefore set forth.

The quantity of liquid may be varied in respect to the amount of solid fuel but I find from experiment that too large an amount of liquid tends to fill the voids and prevent the free passage of air through the mass, while burning and thus give objectionable incomplete combustion and resulting smoke, while too small an amount does not hold the particles together to the desired extent.

15 With the particular liquid above referred to, namely the waste or by-product from the manufacture of heating or illuminating gas, approximately ten gallons of liquid fuel to the ton of dust or screenings gives satisfactory results. Somewhat smaller or larger quantities may be employed.

By the term "coal dust" I do not mean a powder. I use the term with its commercial significance and refer to that product called "screenings" by some coal companies and "coal dust" by others, the product being what is left after the screening out of the various different sizes of commercial coal, such as stove, egg, nut, pea, rice and the larger sizes of buckwheat.

No special apparatus is needed for effecting the mixture of the two ingredients. The mere pouring of the liquid fuel over a pile of the coal dust may be sufficient or it may be sprayed on, or the two may be brought into intimate relationship in various other ways, as for instance by mixing with a shovel or hoe, or by a mechanical mixer, such for instance as is commonly used for the mixing of concrete. The mixture is neither solid nor compressed, so that the entire mass has small cavities or interstitial spaces filled with air and the sides of the coal particles defining this multiplicity of small air chambers are covered or coated with the liquid fuel.

My improved composition may be used in connection with bituminous coal or other solid fuel, the fire bed being first supplied with the usual fuel and then with my improved composition, or the two may be fed together, or my improved composition may

be used alone and the entire fire bed made up of it. It is not necessary to make up the composition in any great quantities as the fireman may mix up merely the day's supply for the furnace or only a ton or so at a time.

This application is a continuation in part and companion of my prior application Serial No. 198,214, filed October 24, 1917.

Having thus described my invention, what I claim as new and desire to secure by Letters Patent is:

1. A fuel composition consisting of loose, 65 commercial anthracite coal-dust or screenings and a high-boiling liquid fuel having low viscosity at ordinary temperatures, the amount of such liquid being merely such as will wet the faces of the coal particles 70 without filling the voids therebetween to a substantial extent and such liquid fuel being of sufficiently high boiling point to insure persistence of a substantial amount of liquid fuel in the mixture until such mixture is at or near the ignition point of the 75 coal.

2. The process which comprises adding to anthracite coal-dust or screenings a liquid fuel of low viscosity and high boiling-point 80 in the quantity which will serve merely to wet the particles of the coal without filling the voids therebetween to a substantial extent, such liquid fuel being in substantial part of sufficiently high boiling point to 85 persist in the mixture up to a temperature near the temperature of ignition of the coal, and then delivering the mixture in loose condition to the fire-bed.

3. A fuel composition consisting of loose 90 commercial anthracite coal dust or screenings, and a liquid fuel having low viscosity at ordinary temperatures, the coal dust and liquid being approximately in the proportions of one ton of the former to ten gallons 95 of the latter, and the liquid fuel being of sufficiently high boiling point to insure persistence of a substantial amount of liquid fuel in the mixture until such mixture is at or near the ignition point of the coal. 100

Signed at New York, on the county of New York, and State of New York, this 11th day of January, 1918.

RICHARD F. DALTON.